# EUROPEAN PATENT SPECIFICATION

(11) **EP 0 326 161 B1**
(45) Date of publication and mention of the grant of the patent: **12.04.1995**
(21) Application number: 89101457.3
(22) Date of filing: 27.01.1989
(51) Int. Cl.: G03C 7/26, G03C 1/825

(54) **Silver halide color photographic materials**
Farbphotographische Silberhalogenidmaterialien
Matériaux photographiques couleurs à l'halogénure d'argent

(30) Priority: 28.01.1988 JP 17771/88
(43) Date of publication of application: 02.08.1989
(73) Proprietor: FUJI PHOTO FILM CO., LTD., Kanagawa 250-01 (JP)
(72) Inventor: Momoki, Yasuhito Fuji Photo Film Co., Ltd., Minami Ashigara-shi Kanagawa (JP); Ohno, Shigeru Fuji Photo Film Co., Ltd., Minami Ashigara-shi Kanagawa (JP)
(74) Representative: Grünecker, Kinkeldey, Stockmair & Schwanhäusser Anwaltssozietät

(56) References cited:
- EP-A- 0 186 169
- EP-A- 0 322 702
- DE-A- 2 521 994
- GB-A- 1 466 836

## Description

This invention relates to silver halide color photographic materials, particularly to silver halide color photographic materials for prints, and more particularly to silver halide photographic materials which give stable color images in long storage, sharp color image quality (which is called sharpness hereinafter), high photographic sensitivity and low photographic fog.

Silver halide color photographic materials are usually spectrally sensitized by adding spectral sensitizers to silver halides according to the subtractive primary colors. A yellow dye-forming coupler, a magenta dye-forming coupler and a cyan dye-forming coupler are contained in the blue-sensitive silver halide emulsion layer, the green-sensitive silver halide emulsion layer and the red-sensitive silver halide emulsion layer, respectively. After conducting imagewise exposure, the silver halide color photographic materials are then processed with a color developing solution comprising an aromatic primary amine color developing agent and then with a bleach-fix bath to obtain an image.

The resulting color image, however, is not always stable to light, heat or moisture. Particularly, the cyan dye image has a larger dark discoloration caused by heat or moisture than both the yellow dye image and the magenta dye image, which changes the color balance. This is a great problem in practical use (for example, the print is turned reddish-brown when preserved in an album).

In order to solve the above problem, JP-A-56-80045 (GB-B-2,066,494; the term "JP-A" as used herein means an "unexamined published Japanese patent application"), JP-A-56-104333 (GB-B-2,068,943), JP-B-57-37857 (US-A-4,333,999) (the term "JP-B" as used herein means an "examined Japanese patent publication"), JP-A-58-105229 (US-A-4,430,423), and JP-A-60-24547 (US-A-4,565,777) teach that couplers substituted at the 2 and 5 positions of the benzene ring of phenol with acyl amino groups, i.e., "2,5-diacylaminophenolic" couplers, are especially excellent as couplers to form very fast cyan-dye images. Also, phenolic cyan couplers having a C₂ or higher alkyl group in the 5-position of phenol can form very fast cyan-dye images.

These phenolic cyan couplers are quite useful for producing color photographic images which are very fast against heat and are preserved well. In addition, it is known that the photographic materials using these couplers are stable in processing and excellent in reproducing colors, particularly because of preservation of cyan density in bleach-fix processing.

Thus the above-mentioned phenolic couplers are favorable compounds to be used as the cyan-dye-forming couplers in color photographic materials.

The standard conditions for selecting the cyan couplers include, for example, light resistance, spectral absorption characteristics of dyes, and effect on photographic properties. Cyan couplers which satisfy all these properties are desired.

On the other hand, another important property needed for color photographic materials for prints is image quality, which is exceedingly influenced by sharpness.

In order to improve the sharpness of color images, the following two techniques are usually used. One is to prevent unsharpening of an image caused by the halation caused by reflecting the light scattered during or after transmission through silver halide emulsion layers on the interface between a silver halide emulsion and a base or on the surface of a photographic material opposite to silver halide emulsion layers and inducing again the reflecting light into the silver halide emulsion layers; and the other is to prevent unsharpening of an image caused by the irradiation caused by the scattering of light on the surface of silver halide in the silver halide emulsion layers.

Silver halide color photographic materials for prints usually employ the method of preventing irradiation.

In order to prevent irradiation, silver halide emulsion layers are colored. Usually, these layers to be colored consist of hydrophilic colloids, therefore, water-soluble dyes are usually contained in the layers for coloring. The dyes should satisfy the following conditions.
(1) The dyes must have the correct spectral absorption fit for the purpose of use thereof.
(2) The dyes must be photochemically inert, i.e., exert no chemical effect on the properties of silver halide photographic emulsion layers, for example, lowering of sensitivity, fading of the latent image and causing photographic fog.
(3) The dyes must be decolored in photographic processing or dissolved and removed to give no undesired color on the processed photographic materials.

In order to find the dyes which satisfy the above conditions, those skilled in the art have eagerly studied and the following dyes have been found, namely, oxonol dyes having pyrazolone or barbituric acid nuclei described in GB-B-506,385; GB-B-1,177,429; GB-B-1,311,884; GB-B-1,338,799; ,GB-B-1,385,371; GB-B-1,467,214; GB-B-1,433,102; and GB-B-1,553,516; JP-A-48-85103 (GB-B-1,373,026); JP-A-49-114420 (GB-B-1,433,102); JP-A-55-161233; JP-A-59-111640; US-A-3,247,127; US-A-3,469,985; and US-A-4,078,933; the other oxonol dyes described in US-A-2,533,472 and US-A-3,379,533; and GB-B-1,278,621; azo dyes described in GB-B-575,691; GB-B-680,631; GB-B-599,623; GB-B-786,907; GB-B-907,125; and GB-B-1,045,609; US-A-4,255,326; and JP-A-59-211043; azomethine dyes described in JP-A-50-100116; JP-A-54-118247; GB-B-2,014,598 and GB-B-750,031; anthraquinone dyes described in US-A-2,865,752; allylidene dyes described in US-A-2,538,009; US-A-2,688,541; and US-A-2,538,008; GB-B-584,609 and GB-B-1,210,252; JP-A-50-40625; JP-A-51-3623; JP-A-51-10927; JP-A-54-118247; JP-B-48-3286 and JP-A-59-37303; styryl dyes described in JP-B-28-3082, JP-B-44-16594, and JP-B-59-28898; triarylmethane dyes described in GB-B-446,583 and GB-B-1,335,422; and JP-B-59-228250; merocyanine dyes described in GB-B-1,075,653; GB-B-1,153,341; GB-B-1,284,730; GB-B-1,475,282; and GB-B-1,542,807; and cyanine dyes described in US-A-2,843,486 and US-A-3,294,539.

Of these dyes, the oxonol dyes having two pyrazolone nuclei have been used for coloring photographic materials as useful dyes which are decolored in a developing solution containing sulfite and exert little harmful influence on photographic emulsions.

However, many of the oxonol dyes having two pyrazolone nuclei have defects of spectrally sensitizing the undesired areas of silver halide emulsions themselves or of the spectrally sensitized silver halide emulsions, causing a decrease of sensitivity, probably because of dropping off spectral sensitizers, and increasing fog.

Moreover, some of them leave after development processing which is conducted more rapidly recently. In order to overcome the problem, it has been proposed to use dyes having high reactivity with sulfite ions, but these dyes have defects that they are not sufficiently stable in dry films to cause the decrease of density after the lapse of time and give no desired photographic effect.

In addition, combinations of the above dyes and thermally fast couplers, for example, the above-mentioned 2,5-diacylaminophenolic couplers, cause the lowering of sensitivity and the increase of fog. This is a great problem in practical use. JP-A-60-225155 discloses that photographic materials prepared by combining 2,5-diacylaminophenolic couplers and specific oxonol dyes have high resistance to dark discoloration, excellent sharpness, good latent image stability and high whiteness (low fog), but it has been found that the above combinations are not satisfactory in respect of sharpness and fog.

From EP-A- 0 186 169 a method for processing light-sensitive silver halide color photographic materials is known comprising carrying out processing of a light-sensitive silver halide color photographic material with a water washing-substitutive stabilizing solution which has been subjected to concentration regulating treatment in the presence of a compound of the following general formula:
wherein R₆ and R₆′ each represent a hydrogen atom, an alkyl group, an aryl group or a heterocyclic group; R₇ and R₇′ each represent a hydroxy group, an alkoxy group, a substituted alkoxy group, a cyano group, a trifluoromethyl group, -COOR₈, -CONHR₈, -NHCOR₈, an amino group, a substituted amino group substituted with an alkyl group having 1 to 4 carbon atoms or a cyclic amino group represented by the formula:
(where p and q each represent 1 or 2, and X represents an oxygen atom, a sulfur atom or -CH₂- ); R₈ represents a hydrogen atom, an alkyl group or an aryl group; L represents a methyne group; n represents 0, 1 or 2; m and m′ each represent 0 or 1.

It is suggested to incorporate into the light-sensitive material for storage stability of cyan dyes a cyan coupler conforming to one of the formulae (III) to (IV) disclosed in this document. EP-A- 0 186 169 thus suggests an improved system for overcoming problems occurring in a processing method wherein a stabilizing solution is used instead of a water washing process.

EP-A- 0 322 702 which represents a state of the art by virtue of Article 54 (3) EPC describes a direct positive photographic material having at least one previously-not-fogged internal latent image-type silver halide emulsion layer on a support having incorporated therein an irradiation-preventing dye and a cyan coupler for preventing a change of photographic performance during preservation and giving images of improved sharpness.

It is the object of the present invention to provide silver halide color photographic materials including light-sensitive silver halide which give stable color images in long storage, high sharpness, high photographic sensitivity and low photographic fog by means of new water-soluble dyes which are easily decolored by processing and stable in storage without exerting any harmful influence on the photographic characteristics of the silver halide emulsion layers.

According to the present invention this object can be attained by a silver halide color photographic material comprising a support having at least one silver halide color photographic emulsion layer coated thereon and containing at least one compound represented by the following general formula (I) and at least one compound represented by the following general formula (II) in at least one hydrophilic colloid layer provided on the support:
wherein each of R₁ and R₂ represents -COOR₅ or
each of R₃ and R₄ represents hydrogen or an alkyl group; each of R₅ and R₆ represents hydrogen, an alkyl group, an aryl group, or R₅ and R₆ together form a 5- or 6-membered ring; each of Q₁ and Q₂ represents an aryl group (2- or 3-valent); each of X₁ and X₂ represents a divalent bonding group or a bond; each of Y₁ and Y₂ represents a sulfonic acid group or a carboxylic acid group; each of L₁, L₂ and L₃ represents a methine group; each of m₁ and m₂ represents 1 or 2; n represents 0, 1 or 2; each of p₁ and p₂ represents 0, 1, 2, 3 or 4; and each of s₁ and s₂ represents 1 or 2;
wherein Y₃ represents -NHCO- or -CONH-; R₈ represents an aliphatic group, an aromatic group, a heterocyclic group or a substituted or unsubstituted aryl amino group; X₃ represents hydrogen, a halogen atom, an alkoxy group or an acylamino group; R₇ represents an alkyl group (containing two or more carbon atoms); and Z represents a hydrogen atom or a group which can be released by coupling with an oxidized developing agent, wherein the photographic material does not contain a previously - not - fogged internal latent image - type silver halide emulsion layer.

In the present invention the terms "alkyl group (or alkyl moiety)", "aryl group (or aryl moiety)", and "aromatic group" each represents substituted and unsubstituted.

The following is a detailed explanation of dyes represented by formula (I).

In formula (I), each of R₁ and R₂ represents -COOR₅ or
each of R₃ and R₄ represents hydrogen or an alkyl group (e.g., methyl, ethyl); each of R₅ and R₆ represents hydrogen, an unsubstituted alkyl group (e.g., methyl, ethyl, isopropyl, butyl); a substituted alkyl group [examples of the substituents include a sulfo group (e.g., sufomethyl, sulfoethyl), a carboxyl group (e.g., carboxymethyl, carboxyethyl), a hydroxy group (e.g., hydroxyethyl, 1,2-dihydroxypropyl), an alkoxy group (e.g., methoxyethyl, ethoxyethyl), a halogen atom [e.g., fluorine, chlorine, bromine (e.g., 2-chloroethyl, 2-bromoethyl, 2,2,2-trifluoroethyl)], a cyano group (e.g., cyanoethyl), an aliphatic or aromatic-sulfonyl group (e.g., methanesulfonylethyl), a nitro group (e.g., 2-nitrobutyl, 2-nitro-2-methylpropyl), an amino group unsubstituted or substituted with an alkyl group such as a methyl group and an ethyl group (e.g., dimethylaminoethyl, diethylaminopropyl), an aryl group (e.g., benzyl, p-chlorobenzyl)]; a phenyl group, and a substituted phenyl group [examples of the substituents include a sulfo group (e.g., p-sulfophenyl, o,p-disulfophenyl), a carboxyl group (e.g., p-carboxyphenyl, m-carboxyphenyl), a hydroxy group (e.g., p-hydroxyphenyl, m-hydroxyphenyl), an alkoxy group (e.g., p-methoxyphenyl, m-ethoxyphenyl), a halogen atom (e.g., p-chlorophenyl, p-bromophenyl, p-fluorophenyl), a cyano group (e.g., p-cyanophenyl, o-cyanophenyl), a nitro group (e.g., p-nitrophenyl, m-nitrophenyl), an amino group unsubstituted or substituted with an alkyl group such as a methyl group and an ethyl group (e.g., p-dimethylaminophenyl, p-diethylaminophenyl), or an alkyl group (e.g., p-methylphenyl, o-methylphenyl)]. When R₁ and R₂ represent -COOR₅ and R₅ represents hydrogen, R₁ and R₂ represent carboxyl groups, which may form not only a free acid but a salt (e.g., sodium salt, potassium salt, ammonium salt, tetraammonium salt).

Also, R₅ and R₆ may form a 5 to 6 membered ring (e.g., morpholino, piperidino). Each of Q₁ and Q₂ represents a 2- or 3-valent unsubstituted aryl group (e.g., phenyl, naphthyl), a 2- or 3-valent substituted phenyl group [examples of the substituents include a C₁ to C₄ alkyl group, a C₁ to C₄ alkoxy group, a halogen atom (chlorine, bromine, fluorine), an aliphatic or aromatic carbamoyl group (e.g., ethylcarbamoyl), an aliphatic or aromatic sulfamoyl group (e.g., ethylsulfamoyl), a cyano group, a nitro group, an alkylsulfonyl group (e.g., methanesulfonyl), an arylsulfonyl group (e.g., benzenesulfonyl), an amino group unsubstituted or substituted with an alkyl group such as a methyl group and an ethyl group (e.g., dimethylamino), an aliphatic or aromatic acylamino group (e.g., acetylamino), and an aliphatic or aromatic sulfonamido group (e.g., methanesulfonamido)]. Q₁ and Q₂ may be bonded with the other moieties at any positions. Each of X₁ and X₂ represents a divalent bonding group and more particularly, -O-,
-SO₂,
or a bond, wherein R₇ represents hydrogen, a C₁ to C₅ alkyl group, or a C₁ to C₅ (total) substituted alkyl group [examples of the substituents include a C₁ to C₃ alkoxy group, a sulfo group (e.g., sulfoethyl, sulfopropyl), a carboxyl group (e.g., carboxylethyl), a cyano group, a hydroxy group (e.g., hydroxyethyl), an amino group unsubstituted or substituted with an alkyl group such as a methyl group and an ethyl group, an aliphatic or aromatic sulfonamido group (e.g., methane sulfonamido), an aliphatic or aromatic carbonamido group (e.g., acetylamino), an aliphatic or aromatic carbamoyl group (e.g., ethylamino carbonyl), and an aliphatic or aromatic sulfamoyl group (e.g., ethylaminosulfonyl)]. Each of Y₁ and Y₂ represents a sulfonic acid group or a carboxylic acid group, which may form not only a free acid but a salt (e.g., sodium salt, potassium salt, ammonium salt, tetraammonium salt). Each of L₁, L₂ and L₃ represents a methine group, or a substituted methine group (where the substituents include a methyl group, an ethyl group and a phenyl group). Each of m₁ and m₂ represents 1 or 2; n represents 0, 1, or 2; each of p₁ and p₂ represents 0, 1, 2, 3 or 4; each of s₁ and s₂ represents 1 or 2.

In the compounds represented by formula (I), each of R₃ and R₄ is preferably hydrogen or a methyl group; each of R₅ and R₆ is preferably hydrogen, a C₁ to C₄ alkyl group, a C₁ to C₆ substituted alkyl group [examples of the substituents preferably include a sulfo group, a carboxyl group, a hydroxy group, a C₁ to C₂ alkoxy group, a chlorine atom, a cyano group, an amino group, and a C₁ to C₄ alkylamino group], a phenyl group or a substituted phenyl group [examples of the substituents preferably include a sulfo group, a carboxyl group, a C₁ to C₄ alkoxy group, a chlorine atom, a cyano group, a C₁ to C₄ alkyl group, an amino group, and a C₁ to C₄ alkyl group, an amino group, and a C₁ to C₄ alkylamino group]. Also, R₅ and R₆ preferably form a 5-membered ring or a 6-membered ring (e.g., a morpholino ring, a pyrolidine ring, a piperidine ring). Each of Q₁ and Q₂ preferably is a phenylene group, a substituted phenylene group [where the substituents preferably include a C₁ to C₄ alkyl group, a C₁ to C₄ alkoxy group, a halogen atom (e.g., chlorine, bromine, fluorine) and a C₁ to C₄ dialkylamino group].

When each of n, m₁, m₂, P₁, P₂, S₁, and S₂ is plural, each set of groups may be the same or different.

Each of X₁ and X₂ preferably represents -O-,
or a bond wherein R₇ preferably represents hydrogen, a C₁ to C₅ alkyl group, or a C₁ to C₅ substituted alkyl group [examples of the substituents include a C₁ to C₃ alkoxy group, a cyano group, a hydroxy group and a C₁ to C₄ alkylamino group].

Moreover, of the dyes represented by formula (I), the most preferred dye is obtained when m₁=m₂=1.

Since the dyes according to the present invention are preferably those which are able to dissolve into a processing solution easily thereby come out from the photographic material, the carbon numbers of an alkyl group and an aryl group preferably are small.

The following are examples of compounds represented by formula (I).

The compounds of formula (I) can be synthesized by various methods, for example, by carrying out the condensation of a pyrazolone represented by formula (III) and a compound represented by formula (IVa), (IVb), (IVc), (IVd) or (IVe) in the presence of bases:

(IVb) HC (OC₂H₅)₃

wherein R₁, R₃, Q₁, X₁, Y₁, L₁, L₂, L₃, m₁, n, p₁ and s₁ have the same definition as given above; Z represents hydrogen, a nitro group, or a halogen atom (e.g., chlorine, bromine); R₈ represents hydrogen, an alkyl group (e.g., methyl, ethyl), or a phenyl group; and X represents an anion (e.g., chloride, bromide, iodide, perchlorate, methyl sulfate, ethyl sulfate, p-toluene sulfonate). The other compounds of those represented by formula (I) can be synthesized by a similar manner to the above-described method.

Examples of bases which are used in the condensation reaction include pyridine, piperidine, triethylamine, triethanol amine, sodium acetate, and potassium acetate.

Examples of solvents which are used for carrying out the condensation reaction include alcohols (e.g., methanol, ethanol, isopropanol), amides (e.g., dimethylformamide, dimethylacetamide, N-methylpyrrolidone), nitriles (e.g., acetonitrile), dimethylsulfoxide, ethylene glycol, ethers (e.g., ethylene glycol monomethylether, ethylene glycol diethylether), water, and a mixture of water and the above-described solvents. The amount of the solvent in the mixture is preferably from 1 to 100 parts by volume per part by volume of water.

The reaction temperature may be selected from the range of from 0°C to the boiling point of the solvent.

The reaction time is decided depending on the reaction temperature, and it is usually selected from the range of from about 30 min to about 3 d.

A pyrazolone represented by formula (III) is used in the condensation reaction in an amount of from 0.1 to 3 mol per mol of a compound represented by formula (IVa), (IVb), (IVC), (IVd) or (IVe).

The following is a description of the synthesis examples for the compounds represented by formula (I).

### Synthesis Example 1 (Compound 3)

To 50 ml of ethanol were added 5.2 g of 3-ethoxycarbonyl-1-(2-sulfobenzyl)pyrazoline-5-one, then 4.2 ml of triethylamine, and 1.5 g of malondialdehyde dianilate. The mixture was heated and refluxed for 3 h to obtain a uniform solution. To this hot solution was added a solution prepared by dissolving 1.2 g of sodium acetate in 15 ml of methanol with stirring. Then, 25 ml of isopropanol were added to the above solution to deposit a dark purple crystal. This crystal was filtered out, washed with isopropanol, and dried to yield 2 g of Compound 3.
Melting point: higher than 300°C
λ$\frac{\text{H₂O}}{\text{max}}$: 551 nm ε: 6.73×10⁴ (ε: extinction exponent)

### Synthesis Example 2 (Compound 8)

A mixture consisiting of 7.4 g of 3-carboxy-1-(2-sulfobenzyl)pyrazoline-5-one, 50 ml of methanol, and 7.5 ml of triethylamine was prepared and cooled with ice. To this mixture were added 2.8 g of glutaraldehyde dianil hydrochloride with stirring for 3 h. To this solution was added a solution prepared by dissolving 4.2 g of sodium acetate in 50 ml of methanol and further 25 ml of isopropanol to deposit a dark purple crystal. This crystal was filtered out, washed with isopropanol, and dried to yield 5.4 g of Compound 8.
Melting point: higher than 300°C
λ$\frac{\text{H₂O}}{\text{max}}$: 626 nm ε: 7.89×10⁴ max

### Synthesis Example 3 (Compound 10)

A mixture consisiting of 8 g of 3-(2-hydroxyethyl carbamoyl)-1-(2-sulfobenzyl)pyrazoline, 30 ml of methanol and 3.8 ml of triethylamine was prepared and cooled. To this solution were added 3 g of glutaraldehyde dianilate and then 2 ml of acetic anhydride. The mixture was reacted at room temperature for 1 h, and then 20 ml of isopropanol were added to deposit a black crystal. The crystal was filtered out, washed with isopropanol, and dried to yield 6.1 g of Compound 10.
Melting point: higher than 300°C
λ$\frac{\text{H₂O}}{\text{max}}$: 633 nm ε: 8.8×10⁴

### Synthesis Example 4 (Compound 18)

A mixture consisting of 8 g of 3-carboxy-1-[2-(4-sulfophenyl)ethyl]pyrazoline-5-one, 50 ml of methanol, and 7 ml of triethylamine was prepared, and then 1.6 g of N,N′-diphenylformamidine hydrochloride were added and heated for 2 h to produce a uniform solution. To this solution were added a solution prepared by dissolving 4.5 g of sodium acetate in 50 ml of methanol and further 20 ml of isopropanol to deposit a yellow crystal. This crystal was filtered out, washed with isopropanol and dried to yield 4 g of Compound 18.
Melting point: higher than 300°C
λ$\frac{\text{H₂O}}{\text{max}}$: 452 nm ε: 2.10×10⁴

### Synthesis Example 5 (Compound 12)

Compound 12 was obtained by using 3-ethoxycarbonyl-1-(2,4-disulfobenzyl)pyrazoline-5-one in the same manner as Synthesis Example 2.
Melting point: higher than 300°C
λ$\frac{\text{H₂O}}{\text{max}}$: 640 nm ε: 7.02×10⁴

### Synthesis Example 6 (Compound 20)

Compound 20 was obtained by using 3-carboxy-1-[2-(4-sulfobutyloxy)benzyl]pyrazoline-5-one in the same manner as Synthesis Example 2.
Melting point: 264 to 269°C (decomposition)
λ$\frac{\text{H₂O}}{\text{max}}$: 628 nm ε: 7.39×10⁴

The compounds which are represented by formula (II) are nondiffusible cyan couplers.

The following is the detailed description of compounds according to formula (II).

In formula (II), R₈ represents a chain or cyclic aliphatic group, preferably having from 1 to 32 (total) carbon atoms (e.g., methyl, butyl, pentadecyl, cyclohexyl), an aromatic group, preferably having from 6 to 32 (total) carbon atoms (e.g., phenyl, naphthyl), a heterocyclic group, preferably 5∼7-membered ring containing at least one of N, O and S atoms as hetero atom (e.g., 2-pyridyl, 3-pyridyl, 2-furanyl, 2-oxazolyl) or a substituted amino group, preferably substituted with at least one of an alkyl and aryl groups. These groups may be substituted by a substituent selected from an alkyl group, an aryl group, an alkoxy or aryloxy group, (e.g., methoxy, dodecyloxy, methoxyethoxy, phenyloxy, 2,4-di-tert-amylphenoxy, 3-tertbutyl-4-hydroxyphenyloxy, naphthyloxy), a carboxyl group, an alkylcarbonyl or arylcarbonyl group (e.g., acetyl, tetradecanoyl, benzoyl), an alkoxycarbonyl or aryloxycarbonyl group (e.g., methoxycarbonyl, benzyloxycarbonyl, phenoxycarbonyl), an aliphatic or aromatic acyloxy group (e.g., acetyl, benzoyloxy, phenylcarbonyloxy), an aliphatic or aromatic sulfamoyl group (e.g., N-ethylsulfamoyl, N-octadecylsulfamoyl), an aliphatic or aromatic carbamoyl group (e.g., N-ethylcarbamoyl, N-methyldodecylcarbamoyl), an aliphatic or aromatic sulfonamido group (e.g., methane sulfonamido, benzenesulfonamido), an aliphatic or aromatic acylamino group (e.g., acetylamino, benzamido, ethoxycarbonylamino, phenylaminocarbonylamino), an imido group (e.g., succinimido, hydantoinyl), an aliphatic or aromatic sulfonyl group (e.g., methanesulfonyl,, a hydroxy group, a cyano group, a nitro group and a halogen atom.

In the specification of the present invention, the term "an aliphatic group" means a straight-chain, branched-chain, or cyclic aliphatic hydrocarbon group, which may be a saturated or unsaturated group such as an alkyl, alkenyl or alkynyl group.

In formula (II), R₇ represents a C₂ to C₂₀ (total) alkyl group (e.g., ethyl, butyl, pentadecyl)

In formula (II), X₃ represents hydrogen, a halogen atom (e.g., Cl, Br, F), an aliphatic group (e.g., methyl, propyl, allyl), an alkoxy group (e.g., methoxy, butoxy), or an aliphatic or aromatic acylamino group (e.g., acetoamide).

In formula (II), Z represents hydrogen or a coupling-releasing group, such as a halogen atom (e.g., fluorine, chlorine, bromine), an alkoxy group (e.g., ethoxy, dodecyloxy, methoxycarbamoylmethoxy, carboxypropyloxy, methylsulfonylethoxy), an aryloxy group (e.g., 4-chlorophenoxy, 4-methoxyphenoxy, 4-carboxyphenoxy), an aliphatic or aromatic acyloxy group (e.g., acetoxy, tetradecanoyloxy, benzoyloxy), an aliphatic or aromatic sulfonyloxy group (e.g., methanesulfonyloxy, toluenesulfonyloxy), an amido group (e.g., dichloroacetylamino, heptabutyrylamino, methanesulfonylamino, toluenesulfonylamino), an alkoxy carbonyloxy group (e.g., ethoxycarbonyloxy, benzyloxycarbonyloxy), an aryloxycarbonyloxy group (e.g., phenoxycarbonyloxy), an aliphatic or aromatic thio group (e.g., ethylthio, phenylthio), a heterocyclic ring thio group (e.g., tetrazolylthio), an imido group (e.g., succinimido, hydantoinyl), and a heterocyclic ring containing at least one N atom (e.g., 1-pyrazolyl, 1-benztriazolyl), an aromatic azo group (e.g., phenylazo). These releasing groups may contain photographically useful groups.

In formula (II), R₇ is preferably a C₂ to C₁₅ alkyl group, more preferably a C₂ to C₄ alkyl group.

In formula (II), Z is preferably hydrogen or a halogen atom, more preferably a halogen atom.

In formula (II), X₃ is preferably a halogen atom.

The compounds represented by formula (II) and synthetic methods thereof are disclosed, for example, in US-A-4,564,590, US-A-2,895,826, US-A-4,557,999, US-A-4,565,777, US-A-4,124,396, US-A-4,613,564, US-A-4,327,173, US-A-4,564,586 and US-A-4,430,423, JP-A-61-39045, JP-A-62-70846, JP-A-61-390441 and JP-A-62-257158.

The following are examples of compounds represented by formula (II) of the present invention.

The dyes of formula (I) can be used as filter dyes, irradiation-preventing dyes or antihalation dyes in any effective amount, preferably in such an amount that the dye provides optical density (of whole hydrophilic colloid layers) of 0.05 to 3.0. The addition thereof is conducted in any step of processing before coating a photographic layer coating composition onto a support.

In order to out spectral absorption which is harmful to spectral sensitizers it is preferable to use a dye represented by formula (I) wherein n=1 for a green sensitizing dye, and a dye represented by formula (I) wherein n=2 for a red sensitizing dye.

The dyes according to the present invention can be dispersed in at least one of hydrophilic colloidal layers, i.e., emulsion layers and the other hydrophilic colloidal layers (intermediate layer, protective layer, antihalation layer including backing layer, and filter layers) by various known methods.
(1) A method of dissolving or dispersing the dyes according to the present invention directly in coating compositions of emulsion layers and hydrophilic colloidal layers, or a method of dissolving or dispersing the dyes according to the present invention in an aqueous solution or a solvent and then using the resulting solution or dispersion in emulsion layers and hydrophilic colloidal layers. The dyes according to the present invention can be dissolved in a suitable solvent, for example, methyl alcohol, ethyl alcohol, propyl alcohol, methyl cellosolve, halogenated alcohol (described in JP-A-48-9715 and US-A-3,756,830), acetone, water, pyridine or mixtures thereof, and the resulting solution may be added to emulsions or a hydrophilic colloidal sulution.
(2) A method of placing a hydrophilic copolymer having the opposite electric charge to the dye ion in layers as a mordant and localizing the dyes in the specific layers by the interaction between the polymer and the dye molecules.
   The term "polymer mordants: means polymers containing secondary and tertiary amino groups, polymers having a nitrogen-containing heterocyclic portion, and polymers containing these quaternary cationic groups, having a molecular weight of 5,000 or more, most preferably 10,000 or more.
   Suitable mordants include, for example, vinyl pyridine polymers and vinyl pyridinium cation polymer described in US-A-2,548,564; vinyl imidazolium cation polymer described in US-A-4,124,386; polymer mordants which are able to cross-link with gelatin, disclosed in US-A-3,625,694; aqueous sol-type mordants disclosed in US-A-3,958,995 and JP-A-54-115228; water-insoluble mordants disclosed in US-A-3,898,088; reactive mordants which can be covalently bonded with the dyes, disclosed in US-A-4,168,976; polymers derived from an ethylenically unsaturated compound having a dialkylaminoalkylester residue as described in GB-B-685,475; products resulting from the reaction of polyvinyl alkylketone and aminoguanidine as described in GB-B-850,281; and polymers derived from 2-methyl-1-vinylimidazole as described in US-A-3,445,231.
(3) A method of dissolving compounds using surfactants. The surfactants may be oligomers or polymers.

A detailed description of the above-described oligomers and the polymers is given in the specification of JP-A-60-158437, pp. 19 to 27. Also the hydrozol of a lipophilic polymer as described in JP-B-51-39835 may be added to the above-obtained hydrophilic colloidal dispersion.

The cyan coupler represented by formula (II) can be employed in an amount of 0.1 to 1 mol, preferably 0.2 to 0.5 mol per mol of silver halide in the photographic silver halide emulsion layer containing the cyan coupler.

The cyan couplers represented by formula (II) are dissolved in high-boiling organic solvents (e.g., phthalic acid ester solvents, phosphate solvents, fatty acid ester solvents) and the resulting solutions are dispersed in hydrophilic colloidal media to be added to silver halide emulsions.

In order to improve the properties of the silver halide color photographic materials in storage, there can be added benzotriazole ultraviolet absorbing agents and substantially water-insoluble, organic solvent-soluble polymers. In particular, the use of these polymers is effective for improving dark discoloration. As the most useful polymers, there are mentioned those described in JP-A- 71262.

The hydrophilic colloids include typically gelatin and also any other conventionally known ones to be used for photographic materials.

The present invention can employ any of silver bromide, silver iodobromide, silver iodochlorobromide, silver chlorobromide, and silver chloride as a silver halide. For the purpose of rapid processing, in particular, silver chlorobromide containing 90 mol% or more of silver chloride (preferably 98 mol% or more) is favorable. This silver chlorobromide may contain a little silver iodide but preferably contains no silver iodide.

The grains of silver halide according to the present invention may be in the form of regular crystals such as a cube and an octahedron or irregular crystals such as a sphere and a tabular or combinations thereof. Also, a mixture of grains having various forms of crystals can be used, but those in the form of regular crystals are preferably used.

The silver halide grains according to the present invention may consist of different phases or a uniform phase as to the inside layer and the surface layer. Also, the grains may be those which form latent images mainly on the surface thereof (e.g., negative emulsion) or mainly in the inside thereof (e.g., internal latent image emulsion, previously fogged direct reversal emulsion). Preferably, the grains are those which can form latent images mainly on the surface thereof.

The silver halide emulsions to be used in the present invention are preferably tabular grain emulsions in which the grains having a thickness of 0.5 »m or less, preferably 0.3 »m or less, a diameter of preferably 0.6 »m or more and an average aspect ratio of 5 or more occupy 50% or more of the whole projected area, or monodisperse emulsions such that the statistical coefficient of variation (a value of s/d̅ obtained by dividing the standard deviation s by a diameter d̅ in the distribution represented by a diameter of a circle approximate to the projected areas) is 20% or less. Also, two or more of tabular grain emulsions and monodisperse emulsions may be mixed.

The photographic emulsions to be used in the present invention can be prepared by the methods described in P. Glafkides, "Chimie er physique Photographique", (Paul Montel Co., Ltd., 1967), G.F. Duffin, "Photographic Emulsion Chemistry" (Focal Press, 1966), and V.L. Zelikman, "Making and Coating Photographic Emulsion" (Focal Press, 1964).

In order to control the growth of grains when forming silver halide grains, there can be used silver halide solvents, for example, ammonia, potassium thiocyanate, ammonium thiocyanate, thioether compounds (e.g., US-A-3,271,157; US-A-3,574,628; US-A-3,704,130; US-A-4,297,439; US-A-4,276,374), thion compounds (e.g., JP-A-53-144319, JP-A-53-82408, JP-A-55-77737), and amine compounds (e.g., JP-A-54-100717).

In the process of forming or physically ripening silver halide grains, there may be present a cadmium salt, zinc salt, thallium salt, iridium salt or complex salt thereof, rhodium salt or complex salt thereof, or ferric salt or ferric complex salt thereof.

Silver halide emulsions are usually chemically sensitized, for example, by the methods described in "Die Grundlagen der Photographischen Prozesse mit Silberhalogeniden" edited by H. Frieser, (Akademisch Verlagsgesellshaft, 1968) pp. 675 to 734.

Namely, there can be used a method of sulphur sensitization using compounds containing sulphur which can react with active gelatin or silver (e.g., thiosulfates, thioureas, mercapto compounds, rhodanines); a method of reduction sensitization using reducible materials (e.g., stannous salt, amines, hydrazine derivatives, formamidine sulfinic acid, silane compounds), and a method of noble metal sensitization using noble metal compounds (e.g., gold complexes and other complexes of metals belonging to Group VIII in the periodic table such as Pt, Ir and Pd) alone or in combination thereof.

In order to prevent photographic fog in the production step, preservation or processing of the photographic materials, or to stabilize the photographic properties, the silver halide photographic emulsions to be used in the present invention can contain various compounds, for example, azoles such as benzothiozolium salt, nitroindazoles, triazoles, benzotriazoles, and benzimidazoles (particularly, those with nitro- or halogen-substituents); heterocyclic mercapto compounds such as mercaptothiazoles, mercaptobenzothiazoles, mercaptobenzimidazoles, mercaptothiadioazoles, mercaptotetrazoles (particularly, 1-phenyl-5-meratptotetrazole), and mercaptopyrimidines; these heterocyclic mercapto compounds having water-soluble groups such as carboxyl group and sulfone group; thioketo compounds such as oxazolinethion; azaindenes such as tetraazindenes (particularly, 4-hydroxy-substituted (1,3,3a,7)tetraazaindenes); benzenethiosulfonic acids; and benzenesulfinic acids as antifoggants or stabilizers.

The silver halide photographic emulsions according to the present invention can contain color couplers such as a cyan coupler, magenta coupler, yellow coupler and compounds for dispersing couplers.

Namely, the silver halide photographic emulsions according to the present invention may contain compounds which form color by oxidation coupling with an aromatic primary amine developing agent (e.g., phenylenediamine derivatives, aminophenol derivatives) in color development. For example, there are 5-pyrazolone couplers, pyrazolobenzimidazole couplers, cyanoacetylcumarone couplers, pyrazolotriazole couplers, and open-chain acylacetonitrile couplers as magenta couplers and acylacetoamide couplers (e.g., benzoyl acetanilides, pivaloyl acetanilides) as yellow couplers.

These couplers are preferably nondiffusible couplers having hydrophobic groups called ballast groups in the molecule. The couplers may be 4 equivalent or 2 equivalent to a silver ion, or colored couplers having the effect of color correction, or couplers releasing development restrainers along with the development (the so-called DIR couplers).

The couplers other than DIR couplers may contain colorless DIR coupling compounds which form colorless products from the coupling reaction and release development restrainers. Also, there may be added ultraviolet absorbing agents and discoloration-preventing agents such as cinnamic acid esters and 2-(2-hydroxyphenyl)benzotriazole.

These discoloration-preventing agents include compounds described in the following patent specifications:
US-A-3,432,300, US-A-3,573,045; US-A-3,574,627; US-A-3,700,455; US-A-3,764,337; US-A-3,935,016; US-A-4,254,216; US-A-4,268,593; US-A-4,430,425; US-A-4,465,757; US-A-4,465,765; US-A-4,518,679; GB-B-1,347,556; GB-B-2,066,975; JP-A-52-152225; JP-A-53-17729; JP-A-53-20327; JP-A-54-145530; JP-A-55-6321; JP-A-55-21004; JP-A-61-72246; JP-A-61-73152; JP-A-61-90155; JP-A-61-90156; and JP-A-61-145554.

The photographic emulsions according to the present invention may contain, for example, polyalkylene oxide or derivatives thereof, such as ether, ester and amine; thioether compounds, thiomorpholines, quaternary ammonium salt compounds, urethane derivatives, urea derivatives, imidazole derivatives and 3-pyrazolidones so as to increase sensitivity and contrast or accelerate development.

The silver halide photographic emulsions according to the present invention can employ known water-soluble dyes (e.g., oxonol dye; hemioxonol dye and merocyanine dye) in addition to the dyes disclosed in the present invention as filter dyes or irradiation-preventing dyes. Also, known cyanine dyes, merocyanine dyes and hemicyanine dyes other than the dyes disclosed in the present invention may be used as spectral sensitizers.

The photographic emulsions according to the present invention may contain various surfactants for the use as coating aids and antistatic agents, improving slipping-propertiers, emulsion-dispersing, preventing adhesion, and improving photographic characteristics (for example, accelerating development, providing high contrast, sensitizing). Also, the photographic materials of the present invention can contain various additives such as discoloration-preventing agents, hardening agents, color antifoggants, ultraviolet-absorbing agents, and protective colloids such as gelatin, which are described particularly in Research Disclosure Vol. 176 (1978, XII) RD-17643.

The finished emulsions are coated on a suitable support, for example, baryta paper, resin-coated paper, synthetic paper, triacetate film, polyethylene terephthalate film, or other plastic supports or glass plates.

The silver halide photographic materials of the present invention include color positive film, color paper, color negative film, color reversal film (which may contain couplers or may not), photographic materials for plate making processes (e.g., lith film, lith dupe film), photosensitive materials for cathode ray tube display (e.g., photosensitive materials for emulsion X-ray recording, direct or indirect photographing materials using a screen), photographic materials for a silver salt diffusion transfer process, photographic materials for a color diffusion transfer process, photographic materials for a dye transfer process, an inhibition transfer process, photographic materials for a silver dye bleach process, photographic materials for recording print-out images, photographic materials for direct printing of images, photographic materials for heat development and photographic materials for physical development.

Exposure for forming photographic images can be carried out by using various well-known light sources, for example, natural light (sun light), or a tungsten lamp, fluorescent lamp, mercury vapor lamp, xenon arc lamp, carbon arc lamp, xenon flash lamp and cathode ray tube flying spot. The exposure time is usually in a range of 1/1000 to 30 s, but can be shorter than 1/1000 s, e.g., in a range of 1/10⁴ to 1/10⁶ s when using a xenon flash lamp or a cathode-ray tube, or longer than 30 s. The spectral composition of light to be used for exposure can be controlled with color filters if desired. Laser rays can be used for exposure. In addition, exposure may be conducted by light excited from phosphors by an X-ray, γ-ray or α-ray.

The photographic processing of the photographic materials of the present invention can be carried out by known processes and processing solutions as described, for example, in Research Disclosure No. 176, pp. 28 to 30 (RD-17643). This photographic processing may be carried out for forming silver images (black and white photographic processing) or color images (color photographic processing). The processing temperature is usually in a range of 18 to 50°C, but may be lower than 18°C or higher than 50°C.

The present invention has no limitation with respect to methods of processing color photographic images. Typically, conventional methods include a method of carrying out exposure, color development, bleach-fixing and, if necessary, washing and stabilizing; a method of carrying out exposure, color development, bleaching, fixing, and if necessary, washing and stabilizing; and a method of carrying out exposure, development with a developing solution containing a black and white developing agent, uniform exposure, color development, bleach-fixing and, if necessary, washing and stabilizing; and a method of carrying out exposure, development with a developing solution containing a black and white developing agent, further development with a color developing solution containing a fogging agent (e.g., sodium borohydride), bleach-fixing, and, if necessary, washing and stabilizing.

The aromatic primary amine color developing agents to be used in the color-developing solutions according to the present invention include those which are known and widely used in various color photographic processes, for example, amino phenolic and p-phenylenediamine derivatives. Preferably, p-phenylenediamine derivatives are used, and the following are the typical examples thereof.
- D-1: N,N-Diethyl-p-phenylenediamine
- D-2: 2-Amino-5-diethylaminotoluene
- D-3: 2-Amino-5-(N-ethyl-N-laurylamino)toluene
- D-4: 4-[N-ethyl-N-(β-hydroxyethyl)amino]aniline
- D-5: 2-Methyl-4-[N-ethyl-N-(β-hydroxyethyl)amino]aniline
- D-6: N-Ethyl-N-(β-methanesulfonamide ethyl)-3-methyl-4-aminoaniline
- D-7: N-(2-Amino-5-diethylaminophenyl ethyl)methanesulfonamide
- D-8: N,N-Dimethyl-p-phenylenediamine
- D-9: 4-Amino-3-methyl-N-ethyl-N-methoxyethylaniline
- D-10: 4-Amino-3-methyl-N-ethyl-N-β-ethoxyethylaniline
- D-11: 4-Amino-3-methyl-N-ethyl-N-β-butoxyethylaniline

Also, these p-phenylenediamine derivatives may be in the form of salts such as a sulfate, hydrochloride, sulfite and p-toluenesulfonate. The above-mentioned compounds are described in US-A-2,193,015, US-A-2,552,241, US-A-2,566,271, US-A-2,592,364, US-A-3,656,950, and US-A-3,698,525. Thse aromatic primary amine color developing agents are used in an amount of about 0.1 g to about 20 g, preferably about 0.5 g to about 10 g per 1 l of a developing solution.

The color developing solutions to be used in the present invention can contain hydroxylamines, as is well known.

Hydroxylamines can be used in the form of free amines in the color-developing solutions, but generally are in the form of aqueous solutions of acid salts, such as sulfate, oxalate, chloride, phosphate, carbonate, and acetate thereof. Hydroxylamines may be substituted or unsubstituterd. The nitrogen atoms of hydroxylamines may be substituted with alkyl groups.

Hydroxylamines are added in an amount of preferably 0 to 10 g, more preferably 0 to 5 g, per 1 l of a color developing solution. As far as the stability of a color developing solution is kept, the smaller amount is better.

As preservatives, there can be added sulfites such as sodium sulfite, potassium sulfite, sodium bisulfite, potassium bisulfite, sodium metasulfite and potassium metasulfite and carbonyl sulfite additives in an amount of preferably 0 g to 20 g per 1 l, more preferably 0 g to 5 g per 1 l. As far as the stability of a color developing solution is kept, the smaller amount is better.

As other preservatives, there are mentioned aromatic polyhydroxy compounds described in JP-A-52-49828, JP-A-56-47038, JP-A-56-32140, JP-A-59-160142, and US-A-3,746,544; hydroxyacetones described in US-A-3,615,503; and GB-B-1,306,176; α-aminocarbonyl compounds described in JP-A-52-143020 and JP-A-53-89425; various metals described in JP-A-57-44148 and JP-A-57-53749; various saccharides described in JP-A-52-102727; hydroxamic acids described in JP-A-52-27638; α,α′-dicarbonyl compounds described in JP-A-59-160141; salicylic acids described in JP-A-59-180588; alkanol amines described in JP-A-54-3532; poly(alkyleneimines) described in JP-A-56-94349; and gluconic acid derivatives as described in JP-A-56-75647. Also hydrazine-N,N-diacetic acid is preferred. These preservatives can be used in a combination of two or more, if desired. Particularly, 4,5-dihydroxy-m-benzenedisulfonic acid, poly(ethylene imine) and triethanol amine are preferably added.

The color developing solutions to be used in the present invention has a pH value of preferably 9 to 12, more preferably 9 to 11, and can contain other compounds known as components of developing solutions.

The detailed description of the kinds and amounts of preservatives, buffers, chelating agents, development accelerators, antifoggants and brightening agents is given in JP-A-63-229457, pp. 11 to 19.

In the present invention the color developing solution are preferably used at a processing temperature in a range of 20 to 50°C, preferably 30 to 40°C, a processing period of time in a range of 20 s to 5 min, preferably 30 s to 4 min, and is replenished in an amount of 30 to 1000 ml, preferably 60 to 400 ml per 1 m² of a photographic material, though the smaller amount is better.

Desilvering process in the present invention is usually conducted as follows. The desilvering process may generally include any of bleaching step-fixing step; fixing step-bleach-fixing step; bleaching step-bleach-fixing step; and bleach-fixing step. The silvering step is carried out for 2 min or less, more preferably for 15 s to 90 s.

The present invention can employ such bleaching solutions, bleach-fixing solutions, fixing solutions, and additives given to the solutions in the amounts described, for example, in JP-A-63-229457, pp. 20 to 25.

Also, washing and/or stabilizing after desilvering can be carried out in the same way as described in said JP-A-63-229457, pp. 25 to 29 line 12.

The present invention is illustrated in greater detail by the following specific Examples. Unless otherwise indicated, all parts, percents and ratios are by weight.

### Example 1

Specimen (1) for multi-layered color print having the following structure of layers was prepared on a paper support laminated with polyethylene on both sides.

### Structure of Layers

The composition of each layer is shown hereinafter. Numerical figures indicate the amounts of coatings (g/m²), and the amounts of silver halide emulsions are calculated in terms of silver. However, the amounts of cyan couplers and dyes are given in mol/m².

### Support

Polyethylene-laminated paper where the polyethylene on the first layer side contained a white pigment (TiO₂) and a blue dye (ultramarine).
The 1st layer (blue-sensitive silver halide emulsion layer)
The 2nd layer (color-mixing-preventing layer)
The 3rd layer (green-sensitive silver halide emulsion layer)
The 4th layer (ultraviolet absorbing layer)
The 5th layer (red-sensitive silver halide emulsion layer)
The 6th layer (ultraviolet absorbing layer)
The 7th layer (protective layer)

The silver halide emulsion (EM-1) used in the above specimen was prepared as follows:
(Solution 1)
(Solution 2)
(Solution 3)
(Solution 4) H₂O was added to equal to 140 ml.
(Solution 5) H₂O was added to equal to 140 ml.
(Solution 6) H₂O was added to equal to 320 ml.
(Solution 7) H₂O was added to equal to 320 ml.

Solution 1 was heated to 74°C, to which solutions 2 and 3 were added. Then, solutions 4 and 5 were added thereto at the same time in 9 min. After further 10 min, solutions 6 and 7 were added at the same time in 45 min. Then the mixed solution was allowed to stand for 5 min after the addition thereof, and then cooled and desalted. Water and dispersion gelatin were added to adjust the pH to 6.2, to obtain a monodisperse cubic silver chlorobromide emulsion having an average particle size of 0.96 »m, a coefficient of variation (a value obtained by dividing standard deviation by an average particle size: s/d̅) of 0.08, and 80 mol% of silver bromide. This emulsion was optimumly chemically sensitized with sodium thiosulfate.

The other silver chlorobromide emulsions (EM-2) to (EM-6) were prepared in a manner similar to the above emulsion (EM-1) except for changing the amounts of chemicals, temperature and time.

The following Table 1 shows the details of these emulsions.

(Soℓv-2) O = P(̵OC₉H₁₉(iso))₃

Specimens (2) to (7) were prepared in the same manner as the above specimen (1) except for changing the dyes of the 4th layer and the cyan coupler of the 5th layer. The compositions of dyes and cyan couplers were shown in Table 2. It is to be noted that the numbers of dyes and cyan couplers correspond to those given in Examples. The following cyan coupler (C) was used for comparison.

Gradation exposure for sensitometry was given to specimens (1) to (7) through a red filter using a sensitometer (FWH type made by Fuji Photo Film Co., Ltd., color temperature of light source: 3200K). In this regard, exposure was carried out for 0.1 s to obtain exposure of 250 CMS. As to sharpness, exposure was given through optical wedge for sharpness to obtain a cyan density of 1.5.

After exposure, the following steps of color development, bleach-fixing, and washing were carried out.

The composition of each processing solution was given as follows:

### Color developing solution

### Bleach-fix bath

The above specimens (1) to (7) were developed and then evaluated as to sensitivity, fogging, sharpness and discoloration. In this regard, the values of relative sensitivity in a density of 1.0 were obtained with using the relative sensitivity value of specimen (1) of 100 for convenience; the values of fogging were obtained in the developing times of 3 min 30 s and also in the forced development time of 7 min; and the values of sharpness were obtained by determining C.T.F. (contrast transfer function) (%) in a spatial frequency of 15 cycles/mm, in which the higher value of sharpness was better. Further, the values of dark discoloration were obtained by leaving each of the developed specimens at 80°C in 70% RH for 14 d and evaluating the percentage of the density obtained in 14 d as to the portion having the color density of 2.0 obtained before the test. The results are shown in Table 3.

As clearly shown in Table 3, the specimens of the present invention prepared by combining cyan couplers and dyes are good photographic materials having high sensitivity, less fogging, high sharpness and good resistance to dark discoloration.

### EXAMPLE 2

Specimen (8) having the following composition was prepared in the same manner as Example 1.
The 1st layer (blue-sensitive silver halide emulsion layer)
The 2nd layer (color-mixing-preventing layer)
The 3rd layer (green-sensitive silver halide emulsion layer)
The 4th layer (ultraviolet absorbing layer)
The 5th layer (red-sensitive silver halide emulsion layer)
The 6th layer (ultraviolet absorbing layer)
The 7th layer (protective layer)

The details of the particles of AgBrCl in the silver halide emulsions used in the above-mentioned specimens are shown in Table 4.

Specimens (8) to (11) were prepared by changing the dyes of the 4th layer and the cyan couplers of the 5th layer in the above specimen. The compositions thereof were shown in Table 5.

The specimens (8) to (11) were exposed to light and treated by the following steps to obtain the evaluation thereof the same as Example 1.

(A 3-tank countercurrent system of rinse (4)→(1) was employed).

The composition of each processing solution is given as follows:

### Color-developing solution

### Bleach-fixing bath

### Rinsing bath

Ion exchange water (each of calcium and magnesium in 3 ppm or less).

The specimens (8) to (11) were developed and evaluated in the same manner as Example 1, with the sensitivity values were obtained when the relative sensitivity of specimen (8) was considered as 100, and the values of fog formed by forced development were obtained when the development time was 90 s. The results are shown in Table 6.

As clearly shown in Table 6, the specimens containing the combinations of cyan couplers and dyes are good photographic materials which have high sensitivity, low fogging values, high sharpness and good resistance to dark discoloration.

### EXAMPLE 3

In order to examine the stability of the dyes of the present invention in the films, the specimens (2), (4), (7), (9) and (11) of Examples 1 and 2 were allowed to stand at 35°C and 80% R.H. for 2 weeks and then evaluated to determine the percentages of the remaining dyes. The results are shown in Table 7.

The result reveals that the dyes according to the present invention have good stability in films.

The present invention can provide silver halide color photographic materials having hydrophilic colloidal layers containing new dyes which are easily decolored by processing and are stable even after the lapse of time without exerting any harmful effect on the photographic properties of photographic emulsions, particularly on sensitivity and fog. Moreover, the present invention can provide silver halide color photographic materials including a red-sensitive emulsion layer which has good resistance to dark discoloration, high sharpness, high sensitivity and low fog.

## Claims

1. A silver halide color photographic material which comprises a support having at least one silver halide color photographic emulsion layer coated thereon and containing at least one compound represented by the following general formula (I) and at least one compound represented by the following general formula (II) in at least one hydrophilic colloid layer provided on the support: wherein each of R₁ and R₂ represents -COOR₅ or each of R₃ and R₄ represents hydrogen or an alkyl group; each of R₅ and R₆ represents a hydrogen atom, an unsubstituted alkyl group, an aryl group or R₅ and R₆ together form a 5- or 6-membered ring; each of Q₁ and Q₂ represents an aryl group; each of X₁ and X₂ represents a divalent bonding group or a bond; each of Y₁ and Y₂ represents a sulfonic acid group or a carboxylic acid group; each of L₁, L₂ and L₃ represents a methine group; each of m₁ and m₂ represents 1 or 2; n represents 0, 1 or 2; each of p₁ and p₂ represents 0, 1, 2, 3 or 4; and each of s₁ and s₂ represents 1 or 2; and wherein Y₃ represents -NHCO- or -CONH-; R₈ represents an aliphatic group, an aromatic group, a heterocyclic group or an aryl amino group which may be substituted; X₃ represents hydrogen, a halogen atom, an alkoxy group or an acylamino group; R₇ represents an alkyl group (containing two or more carbon atoms); and Z represents a hydrogen atom or a group which can be released by coupling with an oxidized color developing agent, wherein the photographic material does not contain a previously - not - fogged internal latent image-type silver halide emulsion layer.

2. A silver halide color photographic material as in claim 1, wherein said compound represented by formula (I) is used in such an amount that the compound provide optical density of 0.05 to 3.0.

3. A silver halide color photographic material as in claim 1 or 2, wherein said compound represented by formula (I) is incorporated in at least one of hydrophilic colloidal layers.

4. A silver halide color photographic material as in any one of claims 1 to 3, wherein the amount of said compound represented by formula (II) is 0.1 to 1 mol per mol of silver halide in the photographic silver halide emulsion layer containing the compound.

5. A silver halide color photographic material as in any one of claims 1 to 4, wherein the alkyl group represented by R₅ or R₆ is substituted with a substituent selected from the group consisting of a sulfo group, a carboxyl group, a hydroxy group, an alkoxy group, a halogen atom, a cyano group, an aliphatic or aromatic-sulfonyl group, a nitro group, an amino group unsubstituted or substituted with an alkyl group, and an aryl group.

6. A silver halide color photographic material as in any one of claims 1 to 4, wherein the aryl group represented by R₅ or R₆ is a phenyl group unsubstituted or substituted with a substituent selected from the group consisting of a sulfo group, a carboxyl group, a hydroxy group, an alkoxy group, a halogen atom, a cyano group, a nitro group, an amino group unsubstituted or substituted with an alkyl group, and an alkyl group.

7. A silver halide color photographic material as in any one of claims 1 to 6, wherein R₁ and R₂ each forms sodium salt, potassium salt, ammonium salt or tetraammonium salt.

8. A silver halide color photographic material as in any one of claims 1 to 7, wherein the aryl group represented by Q₁ or Q₂ represents 2- or 3-valent phenyl or naphthyl group or a phenyl group substituted with a substituent selected from the group consisting of a C₁ to C₄ alkyl group, a C₁ to C₄ alkoxy group a halogen atom, an aliphatic or aromatic carbamoyl group, an aliphatic or aromatic sulfamoyl group, a cyano group, a nitro group, an alkylsulfonyl group, an arylsulfonyl group, an amino group unsubstituted or substituted with an alkyl group, an aliphatic or aromatic acylamino group, and an aliphatic or aromatic sulfonamido group.

9. A silver halide color photographic material as in any one of claims 1 to 8, wherein X₁ and X₂ each represents -O-, or a bond, wherein R₇ represents hydrogen, a C₁ to C₅ alkyl group, or a C₁ to C₅ (total) substituted alkyl group having a substituent selected from the group consisting of a C₁ to C₃ alkoxy group, a sulfo group, a carboxyl group, a cyano group, a hydroxy group, an amino group unsubstituted or substituted with an alkyl group, an aliphatic or aromatic sulfonamido group, an aliphatic or aromatic carbonamido group, an aliphatic or aromatic carbamoyl group, and an aliphatic or aromatic sulfamoyl group.

10. A silver halide color photographic material as in any one of claims 1 to 9, wherein Y₁ and Y₂ each represents a sulfonic acid group or a carboxylic acid group which may form a free acid or a salt.

11. A silver halide color photographic material as in any one of claims 1 to 10, wherein L₁, L₂ and L₃ each represents a methyne group or a methyne group substituted with a substituent selected from the group consisting of a methyl group, an ethyl group, and a phenyl group.

## Patentansprüche

1. Farbfotographisches Silberhalogenidmaterial, umfassend einen Träger, auf den mindestens eine farbfotographische Silberhalogenidemulsion aufgebracht ist, und enthaltend mindestens eine Verbindung, dargestellt durch die folgende allgemeine Formel (I), und mindestens eine Verbindung, dargestellt durch die folgende allgemeine Formel (II), in mindestens einer hydrophilen Kolloidschicht, die auf dem Träger vorgesehen ist: worin R₁ und R₂ jeweils -COOR₅ oder darstellen;
R₃ und R₄ jeweils Wasserstoff oder eine Alkylgruppe darstellen; R₅ und R₆ jeweils ein Wasserstoffatom, eine unsubstituierte Alkylgruppe oder eine Arylgruppe darstellen oder R₅ und R₆ zusammen einen 5- oder 6-gliedrigen Ring bilden;
Q₁ und Q₂ jeweils eine Arylgruppe darstellen; X₁ und X₂ jeweils eine divalente Bindungsgruppe oder eine Bindung darstellen; Y₁ und Y₂ jeweils eine Sulfonsäuregruppe oder eine Carbonsäuregruppe darstellen; L₁, L₂ und L₃ jeweils eine Methingruppe darstellen; m₁ und m₂ jeweils 1 oder 2 darstellen; n 0, 1 oder 2 darstellt; P₁ und P₂ jeweils 0, 1, 2, 3 oder 4 darstellen; und S₁ und S₂ jeweils 1 oder 2 darstellen; und worin Y₃ -NHCO- oder -CONH- darstellt; R₈ eine aliphatische Gruppe, eine aromatische Gruppe, eine heterocyclische Gruppe oder eine Arylaminogruppe, die substituiert sein können, darstellt; X₃ Wasserstoff, ein Halogenatom, eine Alkoxygruppe oder eine Acylaminogruppe darstellt; R₇ eine Alkylgruppe (enthaltend zwei oder mehr Kohlenstoffatome) darstellt; und Z ein Wasserstoffatom oder eine Gruppe darstellt, die durch Kuppeln mit einem oxidierten Farbentwicklungsmittel freigesetzt werden kann,
wobei das fotographische Material keine Silberhalogenidemulsionsschicht vom Typ eines nicht-vorverschleierten latenten Bildes enthält.

2. Farbfotographisches Silberhalogenidmaterial nach Anspruch 1, wobei die Verbindung, dargestellt durch die Formel (I), in solch einer Menge verwendet wird, daß die Verbindung eine optische Dichte von 0,05 bis 3,0 liefert.

3. Farbfotographisches Silberhalogenidmaterial nach Anspruch 1 oder 2, wobei die Verbindung, dargestellt durch die Formel (I), in mindestens eine der hydrophilen Kolloidschichten eingefügt ist.

4. Farbfotographisches Silberhalogenidmaterial nach einem der Ansprüche 1 bis 3, wobei die Menge der Verbindung, dargestellt durch Formel (II), 0,1 bis 1,0 Mol pro Mol Silberhalogenid in der fotographischen Silberhalogenidemulsionsschicht, enthaltend die Verbindung, ist.

5. Farbfotographisches Silberhalogenidmaterial nach einem der Ansprüche 1 bis 4, wobei die Alkylgruppe, dargestellt durch R₅ oder R₆, mit einem Substituenten, ausgewählt aus der Gruppe, bestehend aus einer Sulfogruppe, einer Carboxylgruppe, einer Hydroxylgruppe, einer Alkoxygruppe, einem Halogenatom, einer Cyanogruppe, einer aliphatischen oder aromatischen Sulfonylgruppe, einer Nitrogruppe, einer unsubstituierten Aminogruppe oder einer mit einer Alkylgruppe substituierten Aminogruppe und einer Arylgruppe, substituiert ist.

6. Farbfotographisches Silberhalogenidmaterial nach einem der Ansprüche 1 bis 4, wobei die Arylgruppe, dargestellt durch R₅ oder R₆, eine unsubstituierte Phenylgruppe oder eine mit einem Substituenten, ausgewählt aus der Gruppe, bestehend aus einer Sulfogruppe, einer Carboxylgruppe, einer Hydroxylgruppe, einer Alkoxygruppe, einem Halogenatom, einer Cyanogruppe, einer Nitrogruppe, einer unsubstituierten Aminogruppe oder mit einer Alkylgruppe substituierten Aminogruppe und einer Alkylgruppe, substituierte Phenylgruppe ist.

7. Farbfotographisches Silberhalogenidmaterial nach einem der Ansprüche 1 bis 6, wobei R₁ und R₂ jeweils ein Natriumsalz, ein Kaliumsalz, ein Ammoniumsalz oder Tetraammoniumsalz bilden.

8. Farbfotographisches Silberhalogenidmaterial nach einem der Ansprüche 1 bis 7, wobei die Arylgruppe, dargestellt durch Q₁ oder Q₂, eine 2- oder 3-valente Phenyl- oder Naphthylgruppe oder eine Phenylgruppe, substituiert mit einem Substituenten, ausgewählt aus der Gruppe, bestehend aus einer C₁- bis C₄-Alkylgruppe, einer C₁- bis C₄-Alkoxygruppe, einem Halogenatom, einer aliphatischen oder aromatischen Carbamoylgruppe, einer aliphatischen oder aromatischen Sulfamoylgruppe, einer Cyanogruppe, einer Nitrogruppe, einer Alkylsulfonylgruppe, einer Arylsulfonylgruppe, einer unsubstituierten Aminogruppe oder mit einer Alkylgruppe substituierten Aminogruppe, einer aliphatischen oder aromatischen Acylaminogruppe und einer aliphatischen oder aromatischen Sulfonamidogruppe, ist.

9. Farbfotographisches Silberhalogenidmaterial nach einem der Ansprüche 1 bis 8, wobei X₁ und X₂ jeweils oder eine Bindung darstellen, wobei R₇ Wasserstoff, eine C₁-bis C₅-Alkylgruppe oder eine C₁- bis C₅(gesamt)-substituierte Alkylgruppe mit einem Substituenten, ausgewählt aus der Gruppe, bestehend aus einer C₁- bis C₃-Alkoxygruppe, einer Sulfogruppe, einer Carboxylgruppe, einer Cyanogruppe, einer Hydroxylgruppe, einer unsubstituierten Aminogruppe oder mit einer Alkylgruppe substituierten Aminogruppe, einer aliphatischen oder aromatischen Sulfonamidogruppe, einer aliphatischen oder aromatischen Carbonamidogruppe, einer aliphatischen oder aromatischen Carbamoylgruppe und einer aliphatischen oder aromatischen Sulfamoylgruppe, ist.

10. Farbfotographisches Silberhalogenidmaterial nach einem der Ansprüche 1 bis 9, wobei Y₁ und Y₂ jeweils eine Sulfonsäuregruppe oder eine Carbonsäuregruppe, die eine freie Säure oder ein Salz bilden können, darstellen.

11. Farbfotographisches Silberhalogenidmaterial nach einem der Ansprüche 1 bis 10, wobei L₁, L₂ und L₃ jeweils eine Methingruppe oder eine mit einem Substituenten, ausgewählt aus der Gruppe, bestehend aus einer Methylgruppe, einer Ethylgruppe und einer Phenylgruppe, substituierte Methingruppe darstellen.

## Revendications

1. Matériau photographique couleur à l'halogénure d'argent qui comprend un support portant au moins une couche d'émulsion photographique couleur à l'halogénure d'argent et contenant au moins un composé représenté par la formule générale (I) suivante et au moins un composé représenté par la formule générale (II) suivante dans au moins une couche colloïdale hydrophile disposée sur le support : dans laquelle R₁ et R₂ représentent chacun -COOR₅ ou R₃ et R₄ représentent chacun un atome d'hydrogène ou un groupe alkyle, R₅ et R₆ représentent chacun un atome d'hydrogène, un groupe alkyle non substitué, un groupe aryle ou bien R₅ et R₆ forment ensemble un noyau à 5 ou 6 chaînons ; Q₁ et Q₂ représentent chacun un groupe aryle ; X₁ et X₂ représentent chacun un groupe de liaison divalent ou une liaison ; Y₁ et Y₂ représentent chacun un groupe acide sulfonique ou un groupe acide carboxylique ; L₁, L₂ et L₃ représentent chacun un groupe méthine ; m₁ et m₂ représentent chacun 1 ou 2 ; n représente 0, 1 ou 2 ; p₁et p₂ représentent chacun 0, 1, 2, 3 ou 4 ; et s₁ et s₂ représentent chacun 1 ou 2 ; et dans laquelle Y₃ représente -NHCO- ou -CONH- ; R₈ représente un groupe aliphatique, un groupe aromatique, un groupe hétérocyclique ou un groupe arylamino qui peut être substitué ; X₃ représente un atome d'hydrogène, un atome d'halogène, un groupe alcoxy ou un groupe acylamino ; R₇ représente un groupe alkyle (contenant 2 atomes de carbone ou plus) ; et Z représente un atome d'hydrogène ou un groupe qui peut être éliminé par couplage avec un agent développateur chromogène oxydé, ledit matériau photographique ne contenant pas une couche d'émulsion d'halogénure d'argent du type à image latente interne précédemment non voilée.

2. Matériau photographique couleur à l'halogénure d'argent selon la revendication 1, dans lequel ledit composé représenté par la formule (I) est utilisé en quantité telle que le composé produise une densité optique de 0,05 à 3,0.

3. Matériau photographique couleur à l'halogénure d'argent selon la revendication 1 ou 2, dans lequel ledit composé représenté par la formule (I) est incorporé dans au moins une couche colloïdale hydrophile.

4. Matériau photographique couleur à l'halogénure d'argent selon l'une quelconque des revendications 1 à 3, dans lequel la quantité dudit composé représenté par la formule (II) est de 0,1 à 1 mol par mole d'halogénure d'argent dans la couche d'émulsion d'halogénure d'argent photographique contenant le composé.

5. Matériau photographique couleur à l'halogénure d'argent selon l'une quelconque des revendications 1 à 4, dans lequel le groupe alkyle représenté par R₅ ou R₆ porte un substituant choisi parmi un groupe sulfo, un groupe carboxyle, un groupe hydroxyle, un groupe alcoxy, un atome d'halogène, un groupe cyano, un groupe sulfonyle aliphatique ou aromatique, un groupe nitro, un groupe amino substitué ou non par un groupe aikyle et un groupe aryle.

6. Matériau photographique couleur à l'halogénure d'argent selon l'une quelconque des revendications 1 à 4, dans lequel le groupe aryle représenté par R₅ ou R₆ est un groupe phényle non substitué ou portant un substituant choisi parmi un groupe sulfo, un groupe carboxyle, un groupe hydroxyle, un groupe alcoxy, un atome d'halogène, un groupe cyano, un groupe nitro, un groupe amino substitué ou non par un groupe alkyle et un groupe alkyle.

7. Matériau photographique couleur à l'halogénure d'argent selon l'une quelconque des revendications 1 à 6 dans lequel R₁ et R₂ forment chacun un sel de sodium, un sel de potassium, un sel d'ammonium ou un sel d'ammonium quaternaire.

8. Matériau photographique couleur à l'halogénure d'argent selon l'une quelconque des revendications 1 à 7, dans lequel le groupe aryle représenté par Q₁ ou Q₂ est un groupe phényle ou naphtyle di- ou trivalent ou un groupe phényle portant un substituant choisi parmi un groupe alkyle en C₁-C₄, un groupe alcoxy en C₁-C₄, un atome d'halogène, un groupe carbamoyle aliphatique ou aromatique, un groupe sulfamoyle aliphatique ou aromatique, un groupe cyano, un groupe nitro, un groupe alkylsulfonyle, un groupe arylsulfonyle, un groupe amino non substitué ou substitué par un groupe alkyle, un groupe acylamino aliphatique ou aromatique et un groupe sulfonamido aliphatique ou aromatique.

9. Matériau photographique couleur à l'halogénure d'argent selon l'une quelconque des revendications 1 à 8, dans lequel X₁ et X₂ représentent chacun ou une liaison, dans lesquels R₇ représente l'hydrogène, un groupe alkyle en C₁-C₅ ou un groupe alkyle substitué en C₁-C₅ (au total) ayant un substituant choisi parmi un groupe alcoxy en C₁-C₃, un groupe sulfo, un groupe carboxyle, un groupe cyano, un groupe hydroxyle, un groupe amino non substitué ou substitué par un groupe alkyle, un groupe sulfonamido aliphatique ou aromatique, un groupe carbonamido aliphatique ou aromatique, un groupe carbamoyle aliphatique ou aromatique et un groupe sulfamoyle aliphatique ou aromatique.

10. Matériau photographique couleur à l'halogénure d'argent selon l'une quelconque des revendications 1 à 9, dans lequel Y₁ et Y₂ représentent chacun un groupe acide sulfonique ou un groupe acide carboxylique qui peut former un acide libre ou un sel.

11. Matériau photographique couleur à l'halogénure d'argent selon l'une quelconque des revendications 1 à 10, dans lequel L₁, L₂ et L₃ représentent chacun un groupe méthine ou un groupe méthine substitué par un substituant choisi parmi un groupe méthyle, un groupe éthyle et un groupe phényle.
